# EUROPEAN PATENT SPECIFICATION

(11) **EP 2 045 029 B1**
(45) Date of publication and mention of the grant of the patent: **01.02.2012**
(21) Application number: 08386018.9
(22) Date of filing: 31.07.2008
(51) Int. Cl.: B22F 3/11, C22C 1/04

(54) **Fabrication of aluminium foams by the impregnation of polyurethane foam with a slurry comprising aluminium and salt**
Herstellung von Aluminiumschaum durch die Imprägnierung von Polyurethanschaum mit einem Aluminium und Salz enthaltenden Schlicker
Production d'aluminium mousse par l'impregnation de mousse de polyurethane avec boue comprenant aluminium et sel

(30) Priority: 02.08.2007 GR 20070100504
(43) Date of publication of application: 08.04.2009
(73) Proprietor: ARISTOTLE UNIVERSITY OF THESSALONIKI- Research Committee, 54124 Panepistimioupoli Thessaloniki (GR); Tsipas, Dimitrios, 54124 Thessaloniki (GR); Omar, Mohamad Hidar, 54124 Thessaloniki (GR); Papadopoulos, Dimitrios, 54124 Thessaloniki (GR); Tsipas, Sofia, 54124 Thessaloniki (GR); Michailidis, Nikolaos, 54124 Thessaloniki (GR)
(72) Inventor: Tsipas, Dimitrios, 54124 Thessaloniki (GR); Omar, Mohamad Hidar, 54124 Thessaloniki (GR); Papadopoulos, Dimitrios, 54124 Thessaloniki (GR); Tsipas, Sofia, 54124 Thessaloniki (GR); Michailidis, Nikolaos, 54124 Thessaloniki (GR)
(74) Representative: Petsis, Christos

(56) References cited:
- WO-A-97/31738
- WO-A-02/066693
- US-A- 3 111 396
- US-A- 3 322 535
- US-A- 4 973 385

## Description

The current invention refers to a fabrication method of foams. More specifically the invention aims at the improvement of the fabrication method of Al and its alloys with foams under conditions of atmospheric pressure and leading to final products with improved structures and properties.

Some porous materials are known in materials technology as foams or sponges and these materials are fabricated using different methods,

The advanced materials with porous structures can be found in the group of polymeric, metallic, ceramic and composite materials.

The porous structured materials consist of a group of cells open or closed in structure which leads to much lower density compared to bulk materials. One example of such porous structured material is foams.

Many different methods have been used for fabricating these foams. These methods include liquid metallurgy or powder metallurgy and the pore structure shows a random distribution. This structure is the result of substances (materials) that are added into the mixture and decompose when thermally treated or are produced by the direct introduction of inert gas bubbles into the liquid metal before solidification.

In US Patent No 3111.396 a fabrication method for producing porous materials is presented which includes various consecutive steps in which a solid organic structure is immersed in liquid metal dried and heated in an inert atmosphere until the solid organic template evaporates.

In us patent No 4973.385 a process is given in which gas bubbles are introduced into the liquid metal to produce foaming followed by solidification and the formation of a porous structure.

In the Patent No 9731738 a process is described in which a solution containing alcohol resins, and metal powder is used to impregnate an organic template. The impregnated organic material is dried and heated under vacuum until the organic template is evaporated. The final stage involves sintering of the structure

The advantages of our proposed invention are its simplicity and low cost as it is executed under atmospheric conditions and using standard readily available equipment and its environmentally friendly.

In fig. 1 we present a photo showing the metal foam that was produce using the above described method.

The present invention reports the fabrication of open cell metal foams using organic templates of known 3D geometry. The process involves the step of impregnation of the organic template material with slurry containing alcohol, salts, and Al metal or alloy powder.

The impregnated organic template is left to dry at ambient temperature for 24 hours and the heated at temperature between 215 -500°C for 3.5-5 hours so as to obtain the evaporation of the organic template. The final step includes sintering in an inert atmosphere at temperatures between 500°C-525°C for 0,5-1 hr aiming at producing structures with improved properties.

### Example

97% by weight Al powder 4 microns average size is mixed with 3%AlCl₃. The above mixture is added to ethanol in the ration 1/40 by volume creating slurry.

The template organic material foam is impregnated with the above slurry and left to dry at ambient temperature for 24 hrs. The cell sizes of the organic template foam are selected so as to give the desired size of pores in our final metal foam product.

The slurry impregnated material is placed in a furnace at temperature between 215-500°C for 3,5-5 hrs and using an inert (Ar₂ or N₂) atmosphere so as to limit the formation of oxides. The material is then cooled to room temperature and the final stage involves sintering the metal foam structure in the temperature range 500-525°C for 0.5-1 hr, in an inert atmosphere.

## Claims

1. A method of fabrication of Al and Al alloys foams which involves a selection of the appropriate organic template foams (e.g. polyurethane) with specific cell size and 3D geometry, followed by preparation of a slurry containing Al powder or Al alloy powder, one or more salts (e.g. AlCl₃) and organic material (e.g. alcohol, ethanol, methanol etc.), followed by impregnation of the organic template foam with the slurry or by using auxiliary methods or equipment including the use of vaccum, followed by drying at room temperature for 24 hour, followed by heating between 215°-500°C for 3.5-5 hours in an inert or normal atmosphere until all the organic material is evaporated, followed by cooling to room temperature, and finally sintering the structure at temperatures between 500-525°C for 0.5-1hr in an inert or normal atmosphere.

2. A method according to claim 1 **characterized in that** said salts are halogen containing salts.

3. A method according to claim 1 **characterized in that** the impregnation of the organic template is executed by using auxiliary methods or equipment including the use of vacuum.

4. A method according to claim 1 **characterized in that** a fluidized bed system electric furnace is used.

## Patentansprüche

1. Verfahren zur Herstellung von Schäumen aus Al und Al-Legierungen, welches eine Auswahl geeigneter organischer Template-Schäume (zum Beispiel Polyurethan) mit spezifischer Zellgröße und 3D-Geometrie, gefolgt von einer Präparierung eines Breies, der Al-Pulver oder AL-Legierungspulver, ein oder mehrere Salze (zum Beispiel AlCl₃) und organisches Material (zum Beispiel Alkohol, Ethanol, Methanol, etc.) enthält, gefolgt von einer Imprägnierung des organischen Template-Schaumes mit dem Brei oder durch Verwendung zusätzlicher Verfahren oder Ausrüstung, einschließlich der Verwendung eines Vakuums, gefolgt von einem Trocknen bei Raumtemperatur über 24 Stunden, gefolgt von einem Erwärmen zwischen 215° bis 500°C über 3,5 bis 5 Stunden in einer inerten oder normalen Atmosphäre bis das gesamte organische Material evaporiert ist, gefolgt von einem Abkühlen auf Raumtemperatur und schließlich einem Sintern der Struktur bei Temperaturen zwischen 500 bis 525°C über 0,5 bis 1 Stunde in einer inerten oder normalen Atmosphäre.

2. Verfahren nach Anspruch 1, **dadurch gekennzeichnet, dass** die Salze Halogen enthaltende Salze sind.

3. Verfahren nach Anspruch 1, **dadurch gekennzeichnet, dass** die Imprägnierung des organischen Templates durch Verwenden zusätzlicher Verfahren oder Einrichtungen, einschließlich der Verwendung eines Vakuums ausgeführt wird.

4. Verfahren nach Anspruch 1, **dadurch gekennzeichnet, dass** ein elektrischer Ofen mit einem Fluidbettsystem verwendet wird.

## Revendications

1. Procédé de fabrication de Al et de mousses d'alliage d'Al qui impliquent une sélection génératrice organique appropriée (par exemple du polyuréthane) avec une dimension de cellule et une géométrie 3D spécifique, suivie de la préparation d'une boue contenant de la poudre d'aluminium, ou de la poudre d'alliage d'aluminium, un ou plusieurs sels (par exemple du AlCl₃) et une matière organique (par exemple de l'alcool, de l'éthanol, du méthanol, etc.), suivie de l'imprégnation de la mousse de référence par de la boue, ou par utilisation d'équipement ou de procédés auxiliaires y compris l'utilisation du vide, suivie du séchage à température ambiante pendant 24 heures, suivi d'un chauffage entre 215°C et 500°C pendant 3,5 à 5 heures dans une atmosphère inerte ou normale jusqu'à ce que toutes les matières organiques se soient évaporées, suivie d'un refroidissement à température ambiante, et finalement le frittage de la structure à des températures comprises entre 500 et 525°C pendant 0,5 à 1 heure dans une atmosphère inerte ou normale.

2. Procédé suivant la revendication 1, **caractérisé en ce que** lesdits sels sont des halogènes contenant des sels.

3. Procédé suivant la revendication 1, **caractérisé en ce** l'imprégnation du gabarit 1 la matrice, organique est réalisée par l'utilisation d'équipement ou de procédés auxiliaires y compris l'utilisation du vide.

4. Procédé suivant la revendication 1, **caractérisé en ce qu'**un four électrique à système de lit fluidisé est utilisé.
